

# United States Patent

[11] 3,542,035

[72] Inventor **Wolfgang Dierichs**  
[21] Appl. No. **726,552**  
[22] Filed **May 3, 1968**  
[45] Patented **Nov. 24, 1970**  
[73] Assignee **Henkel & Cie G.m.b.H.**  
[32] Priority **June 5, 1967**  
[33] **Germany**  
[31] **No. H62921**

[54] **TOBACCO FOILS HAVING IMPROVED WET STRENGTH**  
7 Claims, No Drawings  
[52] U.S. Cl. .... **131/15**  
[51] Int. Cl. .... **131/17, 131/140**  
[50] Field of Search. .... **A24b 03/14  
—144, 17; 131/140—144, 15, 17**

[56] **References Cited**  
**UNITED STATES PATENTS**  
3,042,552 7/1962 Rosenberg et al. .... **131/17**  
3,119,812 1/1964 Rogovin et al. .... **260/209**  
3,244,695 4/1966 Schweiger .... **260/209**  
3,353,541 11/1967 Hind et al. .... **131/17**  
3,364,935 1/1968 Moshy et al. .... **131/140**  
3,421,519 1/1969 Moshy et al. .... **131/17**  
3,480,018 11/1969 Fairchild .... **131/17**

*Primary Examiner—Melvin D. Rein  
Attorney—Hammond & Littell*

**ABSTRACT:** This invention relates to a tobacco foil having improved wet strength comprising a dried aqueous mixture of tobacco powder and a water-soluble, film-forming agent, a portion of said water-soluble, film-forming agent consisting of a compound selected from the group consisting of water-soluble xanthan-gum and water-soluble derivatives of xanthan-gum in admixture with a water soluble cellulose ether.

## TOBACCO FOILS HAVING IMPROVED WET STRENGTH

## THE PRIOR ART

It is well known to prepare tobacco foils, which may serve as wrappers for cigars, small cigars or cigarillos, in that tobacco powder is kneaded together with solutions of film-forming, high-molecular weight substances, into a plastic composition, and that this composition is subsequently formed into a film and finally dried. As film-forming materials, for example, natural polysaccharides, such as pectins or plant gums, and above all, cellulose ethers, in particular methylcellulose, or alkali metal salts of the cellulose-glycolic acid have been used.

A considerable disadvantage of the tobacco foils prepared according to these known methods, consists in their low wet strength, because the binding agents employed are water soluble to a high degree, which characteristic they retain even after the foils have been shaped and dried. This fact ensues difficulties during the gluing process, effected with aqueous adhesive solutions, in the production of wrappers for cigars, small cigars or cigarillos. Moreover, the ability to retain the form and the firmness of such wrappers after they become moistened by saliva is very insignificant. Likewise, the tensile strength in the dry condition is not at all satisfactory.

It is furthermore known to improve the wet strength of such foils by an addition of cross-linking agents such as tanning substances or dialdehydes.

According to these processes, the water-soluble, film-forming agents are cross linked and thus they are restricted in their capability to swell up again during admission of water, so that a distinct improvement in their wet strength can be observed.

However, in many cases, the wet strength thus obtained leaves much to be desired, so that the above described difficulties could be eliminated to a certain extent only.

## OBJECTS OF THE INVENTION

An object of the invention is to prepare tobacco foils with greatly improved wet strength, characterized in that they contain, in their function as film-forming agents, xanthan-gum and/or water-soluble derivatives of the xanthan-gum.

Another object of the invention is the obtention of a tobacco foil having improved wet strength comprising a dried aqueous mixture of tobacco powder and a water-soluble, film-forming agent, a portion of said water-soluble, film-forming agent consisting of a compound selected from the group consisting of water-soluble xanthan-gum and water-soluble derivatives of xanthan-gum.

These and other objects of the invention will become more apparent as the description thereof proceeds.

## DESCRIPTION OF THE INVENTION

It has now been discovered that the disadvantages of the prior art can be overcome and the objects of the invention can be achieved by the incorporation into aqueous mixtures of tobacco powder and film-forming agents, of water-soluble xanthan-gum and/or water-soluble derivatives of xanthan-gum and drying the tobacco foils produced from these aqueous mixtures.

The invention, therefore, comprises a tobacco foil having improved wet strength comprising a dried aqueous mixture of tobacco powder and a water-soluble, film-forming agent, a portion of said water-soluble, film-forming agent consisting of a compound selected from the group consisting of water-soluble xanthan-gum and water-soluble derivatives of xanthan-gum.

The water-soluble xanthan-gum is a polysaccharide, composed essentially of glucose, mannose, the potassium salt of the glucuronic acid and acetyl groups in the approximate molar ratio of 2:1:1:1. Furthermore, it contains minor amounts of chemically bonded pyruvic acid. The preparation of xanthan-gum is well known.

Xanthan-gum is prepared in the usual manner by the action of the bacterial strain *Xanthomonas campestris* NRRL-B-1459 on aqueous solutions of glucose or starch and isolation

of the xanthan-gum. Xanthan-gum is a substance easily soluble in water. At a temperature of 20°C., a 2 percent aqueous solution has a viscosity ranging between 2,500 and 6,500 CP. The solutions of xanthan-gum are exceptionally constant with reference to the addition of chemical agents, for example, of mono- or poly-valent salts.

As water-soluble derivatives of the xanthan-gum are to be understood their reaction products with hydroxyalkylating agents, such as ethylene oxide, propylene oxide, butylene oxide, or alkylating agents, such as dimethylsulfate, methylhalide or halocarboxylic acids. Likewise, saponification products belong to this group, as they are obtained, for example, by alkaline deacetylation. These saponification products distinguish themselves by a particularly favorable rheological behavior during the processing.

Advantageously, xanthan-gum or its water-soluble derivatives are not used alone, but in a mixture with water-soluble cellulose derivatives. Suitable for this purpose are all of the film-forming water-soluble cellulose ethers, such as ethylcellulose, hydroxyethylcellulose, ethyloxyethylcellulose, hydroxyethylcellulose containing methyl groups, carboxymethylcellulose, carboxymethylcellulose containing methal or hydroxyethyl groups and still others. Preferably, such mixtures of water and water-soluble cellulose ethers and xanthan-gum or its water-soluble derivatives are used, which have a content of about 3 percent to 60 percent, preferably 6 percent to 50 percent of xanthan-gum or its water-soluble derivatives. Entirely or partly in the place of the water-soluble cellulose derivatives, film-forming, water-soluble starches or their film-forming, water-soluble derivatives can be employed. Preferred are types of water-soluble methyl cellulose, which contain, in addition, hydroxypropyl or hydroxyethyl groups. These types should have a substitution degree of about 1 to 2, and should, in a 2 percent aqueous solution and at a temperature of 20°C., have a viscosity of 200 to 4,000 CP, according to Hoeppler

The amount of water-soluble film-forming agents utilized is that customarily employed in the production of tobacco foils from tobacco powder and water-soluble, film-forming agents.

For the preparation of the tobacco foils of the invention, first of all the water-soluble, film-forming agent is dissolved in water or it is allowed to swell up in water. Next, tobacco powder or, more advantageously, a tobacco powder kneaded in water, is worked onto this solution or gel. The ratio of tobacco powder to the film-forming mixture should be measured so that about 10 to 30 parts by weight of film-forming agents are present per 100 parts by weight of tobacco powder.

In the aqueous mixture, the proportion of solids to water should be measured so that an easily moldable composition is obtained, which can be worked into a smooth foil, for example, by calendering, compressing, pouring, rolling or applying onto any suitable smooth surface by means of a scraper or wiper. The foil obtained in this fashion is then dried at temperatures between about 50°C. and 105°C. However, the water is not totally removed, but the foil is dried to a residual moisture content of about 5 to 20 percent.

In addition, for the execution of the process of the invention, other adjuvants, such as agents for the improvement of the wet strength of the tobacco foil, can be used concomitantly. As is well known, for this purpose natural tanning agents can be employed as, for example, tannins of various origins or catechutannins, catechin, oak or chestnut tannins, ellagic acid or similar combinations. However, in order to obtain an improvement in the wet strength, bivalent aldehydes such as, for example, glyoxal, are preferably used.

Furthermore, in the preparation of these tobacco foils, plasticizing or filling substances are advantageously added. For example, sugar syrup or polyhydric alcohols such as ethylene glycol, glycerin, sorbitol, diethylene glycol, are suitable to be used as plasticizers. Suitable as fillers are kaolin, bentonite, diatomaceous earth or finely distributed silicic acid. If so desired, tobacco fibers, cellulose fibers or glass fibers may be added.

The tobacco foils, obtained according to the process of the invention, are distinguished by a considerably improved wet strength. This wet strength in dry condition is equal or superior to that of the known foils. The foils, prepared according to the process of the invention, can be used as tobacco wrappers for cigars, cigarillos or small cigars, because they do not impair the taste of the tobacco, but effect a favorable influence on the burning of the tobacco goods.

The following examples are illustrative of the invention without, however, being limitative in any respect.

#### EXAMPLES 1—3

One hundred gram of tobacco powder were introduced into 160 g. of water and 5 g. of ethylene glycol. The mixture was then thoroughly kneaded by hand.

In another container, while stirring, 20 g. of binding agents were introduced into 600 g. of water, and the mixture was allowed to stand until it had completely swelled (1—2 hours). Thereafter, while stirring, 8 g. of a 30 percent aqueous glyoxal solution were added. The binding agent consisted of a mixture of methylcellulose (1,000 CP in 2 percent aqueous solution at 20°C., according to Hoeppler) and xanthan-gum (4,000 CP in 2 percent aqueous solution at 20°C., according to Hoeppler). The binding agents for each example had the following quantitative compositions: (1) 18 g. of methylcellulose and 2 g. of xanthan-gum; (2) 16 g. of methylcellulose and 4 g. of xanthan-gum; (3) 12 g. of methylcellulose and 8 g. of xanthan-gum.

In a kneading apparatus used in laboratories, the mixtures, described above and consisting of tobacco powder and the binding agents, were admixed, and, by an addition of citric acid, adjusted to pH 5.6. The batches thus obtained were processed with the aid of a scraper to obtain a thin foil. At a temperature of 100°C. and under air circulation, this foil was dried to a foil sheet of 120 $\mu$  thickness with a moisture content of 15 percent.

For the purpose of testing the wet strength, the foils of 100  $\times$  15 mm. were subjected to a weight load of 200 mg. and suspended to a depth of 50 mm. in water, adjusted to a pH 7 at 20°C. The time, at which the tearing of the foils occurred, was measured as follows:

Example 1, binder 1—6 minutes.  
Example 2, binder 2—20 minutes.  
Example 3, binder 3—25 minutes.

#### EXAMPLES 4—9

One hundred gram of tobacco powder were introduced into a mixture of 160 g. of water and 5 g. of ethylene glycol, and this mixture was thoroughly kneaded by hand.

While stirring, 60 g. of water and 20 g. of a binder were introduced into a second container and the mixture was allowed to stand until it was completely swelled (1—2 hours). Thereafter, under continued stirring, 8 g. of a 30 percent aqueous glyoxal solution were added. The binding agent consisted of a mixture of methylcellulose (1,000 CP in 2 percent aqueous solution at 20°C., according to Hoeppler), and of deacetylated xanthan-gum.

The composition of the binding agents is given in the following table. The first columns indicate the consecutive number of the examples and the amounts of methylcellulose and deacetylated xanthan-gum utilized; the following columns indicate the wet strength and the dry strength measured on the tobacco foils. The working up into foils and determination of the wet strength was effected in the same manner as described

in the preceding examples. The dry strength was determined by means of 10 different samples, each on a conventional tensile-testing apparatus.

TABLE I

| Example   | Methyl-cellulose, g. | De-acetylated xanthan-gum, g. | Wet strength at pH 7 | Dry strength kp./mm.: |
|-----------|----------------------|-------------------------------|----------------------|-----------------------|
| 10 4----- | 18                   | 2                             | 27 minutes.....      | 0.330                 |
| 5-----    | 16                   | 4                             | 80 minutes.....      | 0.330                 |
| 6-----    | 12                   | 8                             | 100 minutes.....     | 0.270                 |
| 7-----    | 10                   | 10                            | 6 days.....          | 0.245                 |
| 8-----    | 4                    | 16                            | 8 days.....          | 0.230                 |
| 9-----    | 0                    | 20                            | <10 days.....        | 0.250                 |

#### COMPARISON TEST

The examples previously described were repeated, however, only the methylcellulose without an addition of xanthan-gum or its derivatives were used as binding agent.

In the same manner as formerly described, the wet strength was measured. The tearing of the foils occurred already after 40 seconds.

This demonstrates the unexpected effect of the presence of water-soluble xanthan-gum or its derivatives in the preparation of tobacco foils from tobacco powder.

The preceding specific embodiments are illustrative of the practice of the invention. It is to be understood, however, that other expedients known to those skilled in the art or disclosed herein may be utilized without departing from the spirit of the invention or the scope of the appended claims.

I claim:

1. A tobacco foil having improved wet strength comprising a dried aqueous mixture of tobacco powder and a water-soluble, film-forming agent in a ratio of from 10 to 30 parts of said water-soluble, film-forming agent to 100 parts of tobacco powder, of said water-soluble, film-forming agent consisting of a mixture of water-soluble cellulose ether and at least 3 percent of said mixture of xanthan-gum selected from the group consisting of water-soluble xanthan-gum and water-soluble derivatives of xanthan-gum, said xanthan-gum being prepared by the action of *Xanthomonas campestris*.

2. The tobacco foil of claim 1 wherein said xanthan-gum is water-soluble deacetylated xanthan-gum.

45 3. The tobacco foil of claim 1 wherein said water-soluble, film-forming agent is a mixture of from 97 percent to 40 percent of a water-soluble cellulose ether and from 3 percent to 60 percent of a compound selected from the group consisting of water-soluble xanthan-gum and water-soluble derivatives of xanthan-gum.

50 4. The tobacco foil of claim 1 wherein said water-soluble, film-forming agent is a mixture of from 94 percent to 55 percent of a water-soluble cellulose ether and from 6 percent to 45 percent of a compound selected from the group consisting of water-soluble xanthan-gum and water-soluble derivatives of xanthan-gum.

55 5. The tobacco foil of claim 3 wherein said water-soluble cellulose ether is a methylcellulose with a substitution degree of about 1 to 2 and with a viscosity of about 200 to 4,000 CP, in a 2 percent aqueous solution at 20°C., according to Hoeppler.

60 6. The tobacco foil of claim 1 comprising a content of a bivalent aldehyde.

65 7. The tobacco foil of claim 6 wherein said bivalent aldehyde is glyoxal.